

Patented Nov. 11, 1952

2,617,768

# UNITED STATES PATENT OFFICE

2,617,768

## LUBRICATING COMPOSITIONS

Wilfred Pohl, Harrow, England, assignor to Shell Development Company, San Francisco, Calif., a corporation of Delaware

No Drawing. Application January 24, 1949, Serial No. 72,557. In Great Britain February 10, 1948

11 Claims. (Cl. 252—33.4)

1

This invention is concerned with lubricating compositions and in particular with lubricating compositions suitable for the lubrication of marine engine bearings.

The lubrication of the bearings of marine engines presents a special problem in that condensed steam, often in considerable quantity, finds its way from the cylinders on to the bearings or at least on to those located below cylinders or piston rods. Accordingly the bearing lubricant employed should function successfully in the presence of water and to this end it should have the property of forming stable water-in-oil emulsions when agitated with water. Furthermore such water-in-oil emulsions, on further addition of water, should not invert to an oil-in-water emulsion. Whereas water-in-oil emulsions tend to adhere to the metallic surfaces to be lubricated and thus maintain a film of lubricant on the surfaces, oil-in-water emulsions tend to drain off the metal surfaces and to be readily washed off by freshly condensed steam and thus result in poor lubrication. Lubricants exhibiting the property of forming stable water-in-oil emulsions which do not invert to oil-in-water emulsions on dilution with water, are hereinafter referred to throughout as "marine engine lubricants."

Marine engine lubricants available in commerce include compositions consisting of a blend of a suitable mineral lubricating oil with an air blown semi-drying fatty oil such as rapeseed oil or fish oil. These air blown semi-drying oils, when used in sufficient quantities, usually 10-20 per cent by weight of the composition, promote the formation of substantially stable water-in-oil emulsions.

The availability of these air blown semi-drying oils however, is frequently restricted to an extent which compels the use of substitute materials. Reduction of the quantity of air blown fatty oil employed ultimately results in lubricating compositions possessing inadequate emulsification and therefore defective lubricating properties. It is an object of the present invention to provide means whereby substantial reduction in the amounts of blown fatty oil incorporated in marine engine lubricants can be effected without adverse effect on their lubricating properties.

2

It has now been discovered that the quantities of these blown fatty oils blended into marine engine lubricants can be substantially reduced and the lubricant nevertheless markedly improved by addition of basic salts of oil-soluble sulfonic acids broadly represented by the general formula

10   
wherein R may be a petroleum hydrocarbon radical, an aliphatic hydrocarbon radical or a mono- or polynuclear aromatic hydrocarbon radical; R' may be one or more alkyl, alkoxy, aroxy, alkyl mercapto, aryl mercapto, alkyl seleno, aryl seleno, alkyl telluro, aryl telluro radicals; Y may be one or more polar radicals such as OH, SH, SeH, TeH, NH<sub>2</sub>, CN, and the like; X is the sulfo radical; the sum of n and x is the valence of the polyvalent metal M, preferably being a divalent metal of the alkaline earth group such as calcium, barium, strontium and magnesium, or the other polyvalent metals such as lead, zinc, tin and aluminum.

15 20 25 Accordingly, the present invention provides marine engine lubricants containing one or more blown fatty oils, and one or more basic sulfonates as broadly defined by the above formula, in amounts sufficient to stabilize and improve the compounded lubricant. The blown fatty oils employed in accordance with this invention are derived from fatty oils of the semi-drying type by blowing air or other oxygen-rich gas through them at an elevated temperature.

30 35 40 45 50 Specifically the fatty oils which are particularly suitable for use in compositions of this invention are: corn oil, cottonseed oil, kapoc oil, rapeseed oil, Ravidon oil, sesame oil, sunflower oil, teaseed oil, rice bran oil, maize oil, as well as semi-drying fish and marine oils, such as whale oil and the like, or mixtures of such oils. These oils may be oxidized by such means as are disclosed in the following U. S. Patents 1,863,004, 2,043,923, 2,156,226, 2,186,910, and 2,216,222. If desired, mixtures of oxidized fatty oils with minor proportions not more than 0.1% in weight, of non-oxidized fatty oils can be used as well as mixtures of the oxidized fatty oils and fatty oils which have been subjected to hydrogenation and/or voltolization treatment. It is to be un-

derstood however, that blown drying-oils such as linseed oil or blown non-drying oils, such as tallow are not included within the scope of the blown fatty oils used in compositions of the present invention. However, minute amounts of non-drying oils such as tallow, lard oil, castor oil, palm oil, and the like, can be admixed with compositions of this invention, if desirable.

The basic metal salts employed in lubricating compositions of this invention are the basic salts of oil-soluble sulfonic acids. Sulfonic acids which are particularly desirable are obtained as by-products arising during the refining of mineral lubricating oil distillates for the production of white oils, transformer oils or medicinal oils or other highly refined oils, by treatment with sulfuric acid, oleum or sulfuryl chloride. Such treatment actually gives rise to two distinct types of naphtha-sulfonic acids, one of which, the so-called "sludge" or "green" acids, is found in the acid sludge and is water-soluble. The present invention is not concerned with salts of acids of this type. The other type of naphtha-sulfonic acids remains in the oil, and, after separation of the acid sludge, can be extracted from the oil by means of alcohol or alcoholic alkali. Sulfonic acid by-products of this latter type, generally known and herein referred to as "oil-soluble naphtha-sulfonic acids," yield basic alkaline earth metal salts useful in the lubricating compositions of this invention. These basic salts are made by conventional methods of neutralization or double decomposition, an excess of the alkaline earth metal compound over that required to form a neutral salt being employed. However, in such conventional processes of preparation, it is possible that a certain amount of neutral salt is formed and the employment of mixtures of basic and neutral salts is within the scope of this invention. Conveniently, the basic alkaline earth metal salt may be formed in situ in the mineral oil to be used as a base for the finished lubricating composition. Thus a suitable mineral lubricating oil may be treated with a sulfonating agent such as sulfuric acid or oleum in the normal way, the oil containing oil-soluble naphtha-sulfonic acids separated from the acid phase and then reacted with an alkaline earth hydroxide such as calcium hydroxide, dry or as an aqueous slurry, in about 100 percent excess of the quantity required to form the neutral sulfonate. This process, after removal of water if present, yields an oil concentrate of the additive which may be blended with further quantities of mineral lubricating oil and with a blown fatty oil to give a lubricating composition falling within the scope of this invention.

Alternatively, the basic alkaline earth salts may be prepared from the sodium salt of an oil-soluble naphtha-sulfonic acid or from a free oil-soluble naphtha-sulfonic acid by treatment with, for example, the hydroxide of an alkaline earth metal in excess of that necessary to form the neutral salt.

Other oil-soluble organic sulfonic acids may also be produced by sulfonating alkyl aromatic hydrocarbons, such as alkyl benzenes, alkyl naphthalenes, alkyl anthracenes, alkyl phenanthrenes, alkyl picenes, alkyl crisenes, alkyl diphenyls, etc. provided the number of carbon atoms in the alkyl chain or chains is sufficient to render the resulting sulfonic acids and their salts soluble in the base. It is desirable that at least one alkyl radical be relatively long, i. e., contain at least 8 or more carbon atoms, not only because of

solubility in oils, but also for the reason that long alkyl chains improve the anti-ring-sticking efficiency of the salts formed with the sulfonic acids thereof. Thus, one may produce an aromatic hydrocarbon suitable for the production of highly efficient sulfonic acids by condensing chlorinated paraffin wax, alkyl chlorides such as octyl, decyl, cetyl, and dodecyl chlorides, fatty alcohols, long-chain olefins such as may be obtained in the cracking of wax, with aromatic hydrocarbons by means of suitable condensing agents such as Friedel-Crafts catalysts, sulfuric acid, phosphorus pentasulfide, phosphoric acid, etc. Sulfonic acids may contain substituent radicals as, for example, paraffin wax substituted naphthalene monosulfonic acids which contain a sulfonic radical attached to one ring of the naphthalene nucleus and a hydroxy or amino radical attached to the other ring. Any of these sulfonic acids may be converted to the basic salt in the manner described above.

Among the basic salts and mixtures thereof which are particularly preferred are:

- 25 Basic calcium salt of oil-soluble petroleum sulfonic acid
- Basic barium salt of oil-soluble petroleum sulfonic acid
- Basic strontium salt of oil-soluble petroleum sulfonic acid
- 30 Basic magnesium salt of oil-soluble petroleum sulfonic acid
- Basic aluminum salt of oil-soluble petroleum sulfonic acid
- Basic calcium salt of alkyl naphthalene sulfonic acid
- Basic calcium salt of diwax benzene sulfonic acid
- Basic barium salt of diwax benzene sulfonic acid
- Basic calcium salt of alkyl phenol sulfonic acid
- Basic calcium salt of diwax thiophenol sulfonic acid
- 40 Basic magnesium salt of diwax thiophenol sulfonic acid
- Basic lead salt of oil-soluble petroleum sulfonic acid
- 45 Basic calcium salt of diwax naphthalene disulfonic acid
- Basic calcium salt of diwax benzene disulfonic acid
- Basic magnesium salt of diwax benzene disulfonic acid
- 50 Basic calcium salt of sulfonated castor oil

The mineral lubricating oils which form the major proportion of my marine engine lubricants may be of any type. Thus they may be derived from paraffinic or asphaltic residues of petroleum oils and they may be refined by any of the many known solvent extraction and/or solvent dewaxing processes or by the conventional methods of acid refining. Blends of different mineral lubricating oils may of course also be employed. A preferred oil is an acid refined oil with a viscosity of about 250 seconds Redwood at 140° F. The natural hydrocarbon oils may be blended with other oleaginous materials of lubricating viscosity, including synthetic lubricants, such as polymerized olefins, copolymers of alkylene glycols and alkylene oxides, organic esters, e. g. 2-ethyl hexyl sebacate, dioctyl phthalate, trioctyl phosphate, polymeric tetrahydrofuran, polyalkyl silicone polymers, e. g. dimethyl silicone polymer, or the synthetic lubricants may be used in place of the natural hydrocarbon oil.

75 In addition to the two additives of this inven-

tion which are admixed with a base oil to form the desired marine engine lubricant, this lubricant may also contain small amounts of other additives such as fatty oils or fats provided that such oils or fats are not of such a nature and are not used in such quantities as to effect adversely the emulsification characteristics of the lubricating compositions. Among such agents may be included acidless tallow, lard oil, oiliness agents, e. g. methyl stearate, extreme pressure agents containing halogen, sulfur and/or phosphorus, oxidation inhibitors such as alkylated phenols and the like.

General formulation of compositions of this invention may be represented as shown in Table I.

## Example IV

96.5 parts acid refined lubricating oil of viscosity 250° Red. at 140° F.

5 3 parts blown fish oil

0.5 part mineral oil solution of mixed basic and neutral calcium salts of oil-soluble naphtha-sulfonic acids containing 11.5 per cent by weight of basic salt, 14.78 per cent by weight of neutral salt and 73.72 per cent by weight of mineral oil

Further illustrative specific combinations of this invention are shown in Table II, each component of which may be used in amounts within the ranges as indicated in Table I.

TABLE II

| Components                                                  | 1 | 2 | 3 | 4 | 5 | 6 | 7 | 8 | 9 | 10 | 11 | 12 |
|-------------------------------------------------------------|---|---|---|---|---|---|---|---|---|----|----|----|
| Blown rapeseed oil                                          | x |   |   |   | x | x |   | x |   |    |    | x  |
| Blown cottonseed oil                                        |   | x |   |   |   |   |   |   |   |    |    |    |
| Blown maize oil                                             |   | x |   |   |   |   |   |   | x |    |    |    |
| Blown whale oil                                             |   |   | x |   |   | x |   |   | x |    |    |    |
| Basic calcium salt of oil-soluble petroleum sulfonic acid   |   |   |   | x |   |   |   |   |   |    |    |    |
| Basic magnesium salt of oil-soluble petroleum sulfonic acid |   | x | x |   |   |   |   | x |   |    | x  | x  |
| Basic barium salt of oil-soluble petroleum sulfonic acid    |   | x |   |   |   |   |   |   | x |    |    |    |
| Basic aluminum salt of oil-soluble petroleum sulfonic acid  | x |   |   |   |   |   |   |   | x |    |    |    |
| Basic calcium salt of diwax benzene sulfonic acid           |   | x |   |   | x |   |   |   |   |    |    |    |
| Basic barium salt of diwax benzene sulfonic acid            |   |   | x |   | x |   | x |   |   |    |    |    |
| Basic barium salt of alkyl naphthalene sulfonic acid        |   |   |   | x | x |   | x |   | x | x  |    |    |
| Acidless tallow                                             | x |   |   |   |   |   |   | x |   | x  |    | x  |
| Voltolized rapeseed oil                                     |   |   |   |   |   |   |   | x | x |    |    |    |

TABLE I

|                                                                    | Broad Range | Limited Range |
|--------------------------------------------------------------------|-------------|---------------|
| Blown fatty oil (semi-drying)                                      | Percent 1-5 | Percent 2.5-5 |
| Basic metal salts of oil-soluble sulfonic acids                    | 0.01-5      | 0.1-0.5       |
| Other agents, e. g. oiliness agents, extreme pressure agents, etc. | 0.1-5       | 0.5-1.5       |
| Base (petroleum hydrocarbon oil and/or synthetic oil)              | Balance     | Balance       |

The following examples are given by way of illustrating the lubricating compositions within the scope of this invention, all parts being parts by weight:

## Example I

96.75 parts acid refined lubricating oil of viscosity 250° Red. at 140° F.  
3 parts blown rapeseed oil  
0.25 parts basic calcium salt of oil-soluble naphtha-sulfonic acids

## Example II

96.75 parts acid refined lubricating oil of viscosity 250° Red. at 140° F.  
3 parts blown fish oil  
0.25 parts basic calcium salt of oil-soluble naphtha-sulfonic acids

## Example III

95.25 parts acid refined lubricating oil of viscosity 250° Red. at 140° F.  
3 parts blown fish oil  
0.25 part basic calcium salt of oil-soluble naphtha-sulfonic acids  
1.5 parts acid free tallow

40 The above compositions can be incorporated with a mineral oil or they can be admixed with synthetic oils or a synthetic oil can be used as a base.

45 With a view to determining the properties and value of the lubricating compositions of this invention, certain laboratory test methods were employed of which the following two are here mentioned, namely the United States Bureau of Ships Emulsion Test (Federal Catalogue 320; 14) and an Inversion Point Test. This latter test is

50 a modification of the United States Bureau of Ships Emulsion Test adapted to determine the point at which a water-in-oil emulsion inverts to an oil-in-water emulsion. The apparatus is that employed in the United States Bureau of Ships Emulsion Test and the procedure is as follows:

55 20 ml. of the oil are placed in the cylinder. The stirrer is started and 0.5 ml. portions of water are added every half minute. After 5 ml. of water have been added, the emulsion is stirred for a

60 further minute and a sample is then examined to ascertain the type of emulsion. After the emulsion has stood for 5 minutes, the stirrer is again started and the above process is repeated for every 5 ml. of water added. An oil suitable for use as a lubricant for marine engine bearings should give a water-in-oil emulsion which does not invert to an oil-in-water emulsion on the addition of 35 ml. of water by the method of this test.

65 70 Table III contains the results obtained when the marine engine lubricants described in the foregoing examples and when some closely related compositions outside the scope of this invention, are subjected to the above two tests.

7 TABLE III 8

| Test No. | Lubricating Composition                                                                  | U. S. Bureau of Ships Emulsion Test | Inversion Point Test                                        |
|----------|------------------------------------------------------------------------------------------|-------------------------------------|-------------------------------------------------------------|
| 1        | As in Example I                                                                          | Stable water-in-oil emulsion.       | Water-in-oil emulsion persists in presence of 35 cc. water. |
| 2        | As in Example II                                                                         | do                                  | Do.                                                         |
| 3        | As in Example III                                                                        | do                                  | Do.                                                         |
| 4        | As in Example I, omitting the basic calcium salt.                                        | Unstable emulsion                   |                                                             |
| 5        | As in Example I, replacing the basic salt by the corresponding neutral salt.             | do                                  |                                                             |
| 6        | The lubricating oil of Example I containing 15 per cent by weight of blown rapeseed oil. | Stable water-in-oil emulsion.       | Water-in-oil emulsion persists in presence of 35 cc. water. |
| 7        | As in Example II, omitting the basic calcium salt.                                       | Unstable emulsion                   |                                                             |

Referring to Table III, a comparison of tests 1, 4 and 6 demonstrates that, although lubricating compositions having the desired properties are obtainable by the simple blending of blown fatty oil with a mineral lubricating oil if the blown fatty oil is present in sufficiently large quantities, the use of small quantities of blown fatty oil results in poor emulsification unless the basic calcium salt is also present. Test 5 illustrates the value of the basic calcium salt specified in Example I, in comparison with the corresponding neutral salt. A comparison of tests 2 and 7 illustrates the beneficial effects of the basic calcium salt on mineral oil compositions containing blown fish oil.

The marine engine lubricants of this invention possess very satisfactory storage stability and substantially no deposition occurs even after long storage at low temperatures, for example, 0° C. Moreover, the compositions are fully compatible with commercial grades of blended lubricants available for use in the lubrication of marine engine bearings.

Although this invention has been described with the particular reference to the use of the lubricating compositions as lubricants for marine engine bearings, the lubricating compositions of this invention can be applied with advantage in other cases where lubrication in the presence of aqueous liquids or water vapor is necessary. Thus, they can be used in the lubrication of pumps and rock drills which have to operate in the presence of water or saline solutions.

In addition to being excellent marine engine lubricants, compositions of this invention may be utilized as flushing oils, rust inhibiting oils, cutting fluids and for various other industrial applications.

I claim as my invention:

1. A marine engine lubricant capable of forming a stable emulsion when in contact with an aqueous medium, containing from 2% to 5% of blown rapeseed oil, 0.1% to 5% of basic alkaline earth metal salt of an oil-soluble petroleum sulfonic acid and the balance being a mineral oil.

2. A marine engine lubricant capable of forming a stable emulsion when in contact with an aqueous medium, containing from 2% to 5% of blown fish oil, 0.1% to 5% of basic alkaline earth metal salt of an oil-soluble petroleum sulfonic acid and the balance being a mineral oil.

3. A marine engine lubricant capable of forming a stable emulsion when in contact with an aqueous medium, containing from 2% to 5% of blown fish oil and from 0.1% to 5% of basic barium salt of oil-soluble petroleum sulfonic acid and the balance being a mineral oil.

4. A marine engine lubricant capable of forming a stable emulsion when in contact with an aqueous medium, containing from 2% to 5% of blown rapeseed oil and from 0.1% to 5% of basic barium salt of oil-soluble petroleum sulfonic acid and the balance being a mineral oil.

5. A marine engine lubricant capable of forming a stable emulsion when in contact with an aqueous medium, containing from 2% to 5% of blown rapeseed oil and from 0.1% to 5% of basic calcium salt of oil-soluble petroleum sulfonic acid and the balance being a mineral oil.

6. A marine engine lubricant capable of forming a stable emulsion when in contact with an aqueous medium, containing from 2% to 5% of blown fish oil and from 0.1% to 5% of basic calcium salt of oil-soluble petroleum sulfonic acid and the balance being a mineral oil.

7. A marine engine lubricant capable of forming a stable emulsion when in contact with an aqueous medium, containing from 2% to 5% of blown semi-drying fatty oil and from 0.1% to 5% of basic alkaline earth metal salt of oil-soluble petroleum sulfonic acid and the balance being a mineral oil.

8. A marine engine lubricating composition containing the following components in the following proportions:

| Parts by weight                                                     |
|---------------------------------------------------------------------|
| Blown rapeseed oil ----- 3                                          |
| Basic calcium salt of oil-soluble naphtha sulfonic acids ----- 0.25 |
| Acid refined mineral lubricating oil ----- Balance                  |

9. A marine engine lubricating composition containing the following components in the following proportions:

| Parts by weight                                                     |
|---------------------------------------------------------------------|
| Blown fish oil ----- 3                                              |
| Basic calcium salt of oil-soluble naphtha sulfonic acids ----- 0.25 |
| Acid refined mineral lubricating oil ----- Balance                  |

10. A marine engine lubricating composition containing the following components in the following proportions:

| Parts by weight                                                     |
|---------------------------------------------------------------------|
| Blown fish oil ----- 3                                              |
| Basic calcium salt of oil-soluble naphtha sulfonic acids ----- 0.25 |
| Acid free tallow ----- 1.5                                          |
| Acid refined mineral lubricating oil ----- Balance                  |

11. A marine engine lubricant capable of forming a stable emulsion when in contact with an aqueous medium, containing from 2% to 5% of blown semi-drying fatty oil and from 0.1% to 5% of basic alkaline earth metal salt of oil-soluble

petroleum sulfonic acid and the balance being a mineral lubricating oil.

WILFRED POHL.

REFERENCES CITED

The following references are of record in the file of this patent:

UNITED STATES PATENTS

| Number    | Name     | Date          |
|-----------|----------|---------------|
| 1,998,767 | MacLaren | Apr. 23, 1935 |
| 2,231,168 | Lazar    | Feb. 11, 1941 |

| Number    | Name      | Date          |
|-----------|-----------|---------------|
| 2,270,577 | Bergstrom | Jan. 20, 1942 |
| 2,470,537 | Waugh     | May 17, 1949  |
| 2,493,483 | Francis   | Jan. 3, 1950  |

OTHER REFERENCES

"Lubrication of Industrial and Marine Machinery," Forbes, John Wiley & Sons, Inc., N. Y., 1945, page 49.  
 "Atlas Surface Active Agents," Atlas Powder Co., copyright 1948, pages 18 and 19.